



US011408048B2

(12) **United States Patent**  
**Xiao**

(10) **Patent No.:** **US 11,408,048 B2**  
(45) **Date of Patent:** **Aug. 9, 2022**

(54) **HIGH-STRENGTH, HOT ROLLED  
ABRASIVE WEAR RESISTANT STEEL STRIP**

(71) Applicant: **TATA STEEL UK LIMITED**, London (GB)

(72) Inventor: **Bin Xiao**, West Midlands (GB)

(73) Assignee: **TATA STEEL UK LIMITED**, London (GB)

(\*) Notice: Subject to any disclaimer, the term of this patent is extended or adjusted under 35 U.S.C. 154(b) by 78 days.

(21) Appl. No.: **16/615,195**

(22) PCT Filed: **May 24, 2018**

(86) PCT No.: **PCT/EP2018/063666**

§ 371 (c)(1),

(2) Date: **Nov. 20, 2019**

(87) PCT Pub. No.: **WO2018/215600**

PCT Pub. Date: **Nov. 29, 2018**

(65) **Prior Publication Data**

US 2020/0157651 A1 May 21, 2020

(30) **Foreign Application Priority Data**

May 24, 2017 (EP) ..... 17172709  
Sep. 22, 2017 (EP) ..... 17192709

(51) **Int. Cl.**

**C21D 9/52** (2006.01)  
**C21D 6/00** (2006.01)

(Continued)

(52) **U.S. Cl.**  
CPC ..... **C21D 9/52** (2013.01); **C21D 6/004** (2013.01); **C21D 6/005** (2013.01); **C21D 6/008** (2013.01);  
(Continued)

(58) **Field of Classification Search**  
CPC ..... C21D 2211/004; C21D 2211/008; C21D 6/005; C21D 8/0205; C21D 8/0226; C21D 8/0263; C21D 9/46; C21D 38/00  
(Continued)

(56) **References Cited**

U.S. PATENT DOCUMENTS

2017/0349987 A1 12/2017 Liu et al.

FOREIGN PATENT DOCUMENTS

EP 2592168 A1 5/2013  
EP 2759615 A1 7/2014  
(Continued)

OTHER PUBLICATIONS

NPL (Hardness conversion table on-line download on 2007). (Year: 2007).\*

(Continued)

*Primary Examiner* — Jie Yang

(74) *Attorney, Agent, or Firm* — Vorys, Sater, Seymour and Pease LLP

(57) **ABSTRACT**

A high strength, hot rolled abrasive wear resistant steel strip with low carbon equivalent values, with a Brinell hardness in the range of 400-465 HBW and a tensile strength in the range of 1180-1500 MPa for strip thicknesses in the range of 3-20 mm, as well as a process for producing such a high strength, hot rolled abrasive wear resistant steel strip.

**14 Claims, 1 Drawing Sheet**



(51) **Int. Cl.**  
*C21D 8/02* (2006.01)  
*C22C 38/02* (2006.01)  
*C22C 38/04* (2006.01)  
*C22C 38/06* (2006.01)  
*C22C 38/42* (2006.01)  
*C22C 38/44* (2006.01)  
*C22C 38/46* (2006.01)  
*C22C 38/48* (2006.01)  
*C22C 38/50* (2006.01)

(52) **U.S. Cl.**

CPC ..... *C21D 8/0205* (2013.01); *C21D 8/0226* (2013.01); *C21D 8/0263* (2013.01); *C22C 38/02* (2013.01); *C22C 38/04* (2013.01); *C22C 38/06* (2013.01); *C22C 38/42* (2013.01); *C22C 38/44* (2013.01); *C22C 38/46* (2013.01); *C22C 38/48* (2013.01); *C22C 38/50* (2013.01); *C21D 2211/004* (2013.01); *C21D 2211/008* (2013.01)

(58) **Field of Classification Search**  
USPC ..... 148/320  
See application file for complete search history.

(56) **References Cited**

FOREIGN PATENT DOCUMENTS

|    |            |    |         |
|----|------------|----|---------|
| EP | 3235923    | A1 | 10/2017 |
| JP | 2012077336 | A  | 4/2012  |
| WO | 2016095720 | A1 | 6/2016  |

OTHER PUBLICATIONS

International Search Report and Written Opinion dated Jun. 20, 2018 for PCT/EP2018/063666 to Tata Steel UK Limited filed May 24, 2018.

\* cited by examiner



## HIGH-STRENGTH, HOT ROLLED ABRASIVE WEAR RESISTANT STEEL STRIP

### CROSS-REFERENCE TO RELATED APPLICATIONS

This is a § 371 National Stage Application of International Application No. PCT/EP2018/063666 filed on May 24, 2018, claiming the priority of European Patent Application No. 17192709.8 filed on Sep. 22, 2017 and European Patent Application No. 17172709.2 filed on May 24, 2017.

### FIELD OF THE INVENTION

The invention relates to a high strength, hot rolled abrasive wear resistant steel strip and a process for producing such a strip.

### BACKGROUND OF THE INVENTION

Hot rolled abrasive wear resistant steel products are typically used in harsh abrasive environments, such as in lifting and excavating applications. Typically the aim of the end users is to extend the service life of these abrasive wear resistant as much as possible in order to reduce maintenance/ downtime and therewith the costs.

There is a very strong correlation between the abrasion resistance and the surface hardness of steel, thus to further improve the durability of these abrasive wear resistant steel products, high strength, high hardness as well as high wear resistant properties are required. Therefore, hot rolled martensitic steels with high hardness and desired impact toughness are extensively used in the lifting and excavating industry.

With the continuing development of hot rolled abrasive wear resistant steel strip over the years and a demand for longer service time, the Brinell hardness has been steadily increased resulting in a Brinell hardness of 400 HBW and higher. The general notation to identify the abrasive-resistant steel grades is to classify them according to their surface hardness in terms of Brinell hardness (HBW), and the most common grades are 400 HBW, 450 HBW and 500 HBW. With the increase of the Brinell hardness of the abrasive wear resistant steel strip, such as increasing from 400 HBW to 500 HBW, also the carbon equivalent values (CEV, CET and Pcm) have increased to achieve required hardness and improve hardenability in thicker hot rolled strips, that is in particular with thicknesses of 10 mm and more. This means that even for the same steel grade, such as 400 HBW, different steel composition are needed for the thicker steel strips than for abrasive wear resistant steel strip of less than 10 mm thickness.

Because of the necessary high carbon equivalent values to increase hardness and improve hardenability the different steel compositions used for thicker hot rolled strip have a number of disadvantages. Important properties relating to the processing of these wear resistant hot rolled strip, such as cutting, drilling, bending and welding of the steel strip, deteriorate in comparison with thinner steel strip with lower carbon equivalent values. This results in difficult processing steps with the manufacturing of abrasive wear resistant steel products, which is in particular the case with more complicated products, increasing the costs significantly. To solve this issue, a novel steel composition is designed to have strong strengthening mechanisms to obtain required hardness in thicker strips without increasing the carbon equivalent values noticeably, also the fast and controllable water

cooling rate on the run-out table on the hot mill are key factors to produce 400 HBW and 450 HBW grades of hot rolled wear resistant strips that have a thickness in the range of 3-20 mm.

### OBJECTIVES OF THE INVENTION

It is an objective of the present invention to provide a high strength, hot rolled abrasive wear resistant steel strip with a Brinell hardness of above 400 HBW and low carbon equivalent values.

It is another objective of the present invention to provide a high strength, hot rolled abrasive wear resistant steel strip with a Brinell hardness of above 400 HBW and low carbon equivalent values with a minimum thickness of 3 mm.

It is another objective of the present invention to provide a high strength, hot rolled abrasive wear resistant steel strip with a Brinell hardness of above 400 HBW and low carbon equivalent values with a thickness in the range of 3-20 mm with a single chemistry composition.

It is another objective of the present invention to provide a high strength, hot rolled abrasive wear resistant steel strip with high impact toughness.

It is another objective of the present invention to provide a high strength, hot rolled abrasive wear resistant steel strip which has good bendability properties.

It is another objective of the present invention to provide a high strength, hot rolled abrasive wear resistant steel strip that can easily be welded.

It is another objective of the present invention to provide a high strength, hot rolled abrasive wear resistant steel strip with high wear resistant.

### BRIEF DESCRIPTION OF THE DRAWINGS

FIG. 1 shows a SEM image.

### DESCRIPTION OF THE INVENTION

The invention relates to a high strength, hot rolled abrasive wear resistant steel strip with a Brinell hardness of above 400 HBW and low carbon equivalent values and a process for producing such high strength, hot rolled abrasive wear resistant steel strip.

One or more of the objectives of the invention are realized by providing a high strength, hot rolled abrasive wear resistant steel strip, wherein the strip has a thickness in the range of 3-20 mm and has a microstructure comprising martensite, auto-tempered martensite with iron carbides and NbC, Nb(C, N) and NbV(C, N) particles and trace amounts of retained austenite in martensite-austenite islands, with low carbon equivalent values and wherein the steel contains in weight percentages:

C: 0.13-0.29  
Si: 0.01-0.05  
Mn: 0.5-1.4  
Cr: 0.05-0.8  
Mo: 0.05-0.4  
Ni: at most 0.1  
Cu: at most 0.1  
Al: 0.01-0.08  
Ti: at most 0.02  
B: at most 0.004  
Nb: 0.005-0.035  
V: 0.03-0.20  
P: at most 0.020  
S: at most 0.010

N: at most 0.006

H: at most 0.0004

Ca additions for sulphide shape control: 0.0005-0.005  
wherein the total content of Nb+V is in a range of  
0.035-0.16

other elements in amounts of impurity level, balance iron,  
and

wherein CEV is at most 0.46, CET at most 0.34 and Pcm  
at most 0.32, and

wherein the strip has a Brinell hardness of at least 400  
HBW and a tensile strength of at least 1316 MPa.

Carbon is the most important element for increasing the  
hardness and hardenability of martensite. It also improves  
the strength and wear resistant of the steel strip. In order to  
ensure that the room temperature surface Brinell hardness  
and the centre Vickers hardness of the hot rolled strip up to  
20 mm are sufficient, the C content is set to not less than 0.13  
wt % but not more than 0.29 wt % and preferably in the  
range of 0.15-0.23 wt %.

Silicon Si acts as a deoxidiser for steelmaking, and Si is  
an important element for the present invention. The Si  
content is at the least 0.01 wt % but less than 0.05 wt % in  
order to get very good surface quality of the hot rolled steel  
strip. Good surface quality is realised because much less red  
oxide scales are produced at such low Si content.

Mn increases hardenability of steel and lowers the critical  
or minimum cooling rate on the run-out table for the  
martensite formation. However, high levels of Mn do result  
in high CEV, CET and Pcm levels, which reduces weldability,  
and promote the harmful banding segregation and  
adversely affect the homogeneity of the microstructure. In  
the present invention, the Mn content is controlled at the  
0.5-1.4 wt %, and more preferably in the range of  
0.6-0.9 wt %.

Cr also enhances the hardenability of the steel and reduces  
the critical cooling rate for the martensite formation, also Cr  
can replace Mn content partly to reduce the segregation  
tendency. However, high levels of Cr do result in poor  
performance in weldability, thus the Cr content should be in  
a range of 0.05 to 0.8 wt % or in a more limited range of 0.05  
to 0.6 wt %.

Molybdenum Mo can increase quench hardenability of  
steel significantly and increase hardness of hot rolled strip,  
also increase tempering resistant. However, higher content  
of Mo will increase cost and the carbon equivalent values  
(CEV, CET and Pcm) remarkably, thus the Mo content  
should be in a range of 0.05 to 0.4 wt %. The Mo content will  
typically be in a range of 0.05-0.25 wt %, or in a range of  
0.1-0.25 wt %.

Niobium Nb is a very important micro-alloying element  
in the present invention because Nb can be a useful addition  
below 0.05 wt %. NbC and/or Nb (CN) particles (to fix  
some solute N) will be present during the hot forming  
operation which will help to pin austenite grain boundaries  
to prevent undesirable austenite grain growth, and hence  
promote a fine microstructure in the final product. Also the  
remaining Nb in solid solution at the hot forming temperature  
can increase hardenability by reducing transformation  
temperatures. Further during cooling Nb is able to form fine  
precipitates which could contribute to strength and toughness.  
However, a high content of Nb will increase the  
production cost so typically Nb is kept in a range of 0.005  
to 0.035 wt %. Nb will typically be in a range of 0.01 to  
0.035 wt % or 0.015 to 0.030 wt %.

Vanadium is another important micro-alloying element in  
the present invention, and V has a similar but less powerful  
effect as Nb. The addition of both Nb and V further strength-

ens the hot rolled steel by forming fine Nb and V carbides,  
nitrides and carbo-nitrides. The addition of V should be  
within a range of 0.03-0.20 wt %, and will typically be in a  
range of 0.03-0.15 wt % or 0.03-0.12 wt %. With both Nb  
and V added into the steel to optimise the strength and  
toughness level, the content of Nb+V is in the range of  
0.06-0.16 wt % and typically in a range of 0.06-0.12 wt %.

Aluminium acts as a strong deoxidisation element to keep  
the oxygen content as low as possible. Further, Al is com-  
bined with free nitrogen N to form AlN precipitates, which  
can improve the strength, and helps to prevent that boron  
reacts with nitrogen to form BN precipitates. The Al content  
should be in the range of 0.01-0.08 wt % and is typically in  
the range 0.03-0.07 wt %.

Titanium is also combined with carbon and/or nitrogen to  
form TiC, TiN and/or Ti(C,N) particles, which suppresses  
austenite grain coarsening during the high temperature  
reheating stage. However, the large TiC, TiN and/or Ti(C,N)  
particles are undesirable for the Charpy toughness. There-  
fore, the Ti content in the present invention should be at most  
0.02 wt % and preferably at most 0.01 wt %.

Boron can be effective in promoting higher strength  
phases such as martensite, by retarding the formation of  
ferrite during phase transformation on the run out table. The  
use of Boron could allow a reduction in some of the other  
alloying elements, resulting in reduced alloying costs and  
lower carbon equivalent values (CEV, CET and Pcm). It is  
also important to minimise the formation of BN as this will  
reduce the "free" boron content for increasing the harden-  
ability. The roles of Ti and Al in the composition according  
to the present invention is to protect the "free" boron content  
because Ti and Al can form TiN and AlN respectively, so that  
only a minimum amount of "free" N can be combined with  
Boron to form undesired BN. Therefore, Boron content  
should be in the range of 0.0005 wt % to at most 0.0040 wt %.

Expensive elements such as Cu and Ni could be consid-  
ered as further strengthening additions, but their effect on  
strength is relatively modest, and they could only be used in  
limited amounts to avoid increasing the CEV, CET and Pcm  
too much. For that reason the content of each of these  
elements is at most 0.1 wt %.

Calcium additions are added for the Ca treatment of the  
steel to control sulfide shape and composition; this results in  
a modification to the MnS inclusions, resulting in an  
improved Charpy toughness but also improving processabil-  
ity. Other potential improvements associated with Ca addi-  
tions (and low S) would be a reduction of welding defects  
such as lamellar tearing. Typical amount of Ca in the  
invention is 0.0005 to 0.005 wt %. However, when Ca is  
added excessively, the effect is saturated and the economic  
efficiency is reduced. Therefore, it is better to Ca level below  
0.005 wt %.

P and S must be controlled to low levels to allow good  
Charpy toughness and weldability to be achieved, and to  
allow defect free slabs to be produced for rolling to strip.

With this composition the problem of high carbon equiva-  
lent values (CEV, CET and Pcm) for higher wear resistant  
steel grade and in particular strip thicknesses above 10 mm  
is solved in which these values are kept below certain  
maximum values. With the wear resistant steel strips accord-  
ing the prior art these values are higher for the higher wear  
resistant steel grade and for the thicker strips in order to  
realise the required hardness and hardenability for these  
higher steel grade and thicker hot rolled strips.

With the above composition the values for the different  
carbon equivalents are respectively CEV≤0.46, CET≤0.34,

## 5

and  $P_{cm} \leq 0.32$ , and more preferably  $CEV \leq 0.46$ ,  $CET \leq 0.33$ , and  $P_{cm} \leq 0.31$ , wherein the carbon equivalent equations for  $CEV$ ,  $CET$  and  $P_{cm}$  values are:

$$CEV = C + Mn/6 + Cr/5 + Mo/5 + V/5 + Cu/15 + Ni/15;$$

$$CET = C + Mn/10 + Mo/10 + Cr/20 + Cu/20 + Ni/40$$

$$P_{cm} = C + Si/30 + Mn/20 + Cu/20 + Cr/20 + Mo/15 + V/10 + Ni/60 + 5B$$

An advantage of low carbon equivalent values is that additional weld processing steps such as pre-heating can be avoided, thus reducing fabrication costs.

According to a further aspect the  $CEV$  is at most 0.43 and/or  $CET$  at most 0.31 and/or  $P_{cm}$  at most 0.29.

The strip with the above composition has a microstructure which comprises martensite, auto-tempered martensite with iron carbides and  $NbC$ ,  $Nb(C, N)$  and  $NbV(C, N)$  particles. The microstructure further comprises trace amounts of retained austenite in martensite-austenite (MA) islands. The volume fractions of the martensite content including auto-tempered martensite and MA islands, and lower bainite are depending on the target steel grades and strip thickness. In a typical sample the volume fraction of martensite including auto-tempered martensite and MA islands is  $85 \pm 3\%$ , and the rest of microstructure is lower bainite that is  $15 \pm 3\%$  in volume fraction.

According to a further aspect a process is provided for producing a high strength, hot rolled abrasive wear resistant steel strip, wherein the strip has a thickness in the range of 3-20 mm and has a microstructure comprising martensite, auto-tempered martensite with iron carbides and  $NbC$ ,  $Nb(C, N)$  and  $NbV(C, N)$  particles and trace amounts of retained austenite in martensite-austenite islands, comprising the steps of:

casting a slab with a composition in wt %

C: 0.13-0.29

Si: 0.01-0.05

Mn: 0.5-1.4

Cr: 0.05-0.8

Mo: 0.05-0.4

Ni: at most 0.1

Cu: at most 0.1

Al: 0.01-0.08

Ti: at most 0.02

B: at most 0.004

Nb: 0.005-0.035

V: 0.03-0.20

P: at most 0.020

S: at most 0.010

N: at most 0.006

H: at most 0.0004

Ca additions for sulphide shape control: 0.0005-0.005

and wherein the total content of  $Nb + V$  is in a range of 0.035-0.16,

other elements in amounts of impurity level, balance iron, containing the slab in a hot box for a predefined time, reheating the slab to a temperature of at least  $1150^\circ C$ , keeping the slab for a predefined period at the temperature of at least  $1150^\circ C$ , and

hot rolling the slab to a hot rolled steel strip with a finish

rolling temperature in the range of  $800-940^\circ C$ , water cooling the strip with a cooling rate in the range of  $-20-150^\circ C/s$ ,

coiling the strip at a temperature in the range of  $100-250^\circ C$ .

## 6

The slab with the above composition is cast as a slab within a thickness range of 200 to 300 mm from the continuous casting process, or from the thin slab casting process. After casting the hot slab with a maximum temperature in a range of  $500-600^\circ C$ , is contained in the hot box and slowly cooled down for a period in the range of 2-6 days, preferably 3-5 days. The temperature in the hot box is kept at a temperature in a range of  $400-500^\circ C$ . This is a very critical step in the process for the hydrogen diffusing out of the slab so that the hydrogen content is less than 1 ppm to minimise the hydrogen embrittlement cracking in such high strength wear resistant steel.

Typically the temperature of the as-cast slab at the end of the period in the hot box is in the range of  $400-500^\circ C$ . After 15 this period in the hot box the slab is reheated to at least  $1150^\circ C$ , and is kept at the temperature of at least  $1150^\circ C$  for a period of up to 3 hours prior to hot rolling. The initial rough 20 rolling is taking place above recrystallization stop temperature ( $T_{nr} > 1050^\circ C$ ) to obtain fine recrystallized grain, while for the finish rolling is performed below  $T_{nr}$  with reduction more than 60% to form heavy deformed pancaked austenite 25 grain size, and the end of finish rolling temperature is in the range  $800-950^\circ C$ . The final thickness of the hot rolled strip is in the range of 3-20 mm.

Immediately after hot rolling, the time between the end of the hot rolling step and the cooling step is kept as short as possible and is preferably less than 10 seconds, and more preferably less than 5 seconds. The thin/thick strip is water 30 cooled on the run-out table with a first defined cooling rate between 40 and  $150^\circ C/s$  for the 450 HBW grade and between 30 and  $70^\circ C/s$  for the 400 HBW from above to the martensite start temperature ( $Ms$ ) and from the  $Ms$  with second defined cooling rate between 25 and  $60^\circ C/s$  for the 450 HBW grade and between 20 and  $30^\circ C/s$  for the 400 35 HBW to a low coiling temperature in the range of  $100-250^\circ C$ , more preferably in the range of  $100-200^\circ C$ , to ensure its high strength and high hardness. By decreasing the allowable coiling temperature range the homogeneity of the microstructure will improve.

40 In this important run-out table cooling, the critical fast water cooling rate above martensite start temperature ( $Ms$ ), and the minimum defined cooling rate ( $> 25^\circ C/s$  for the 450 HBW steel grade and ( $> 20^\circ C/s$  for the 400 HBW steel grade) between the  $Ms$  and coiling temperature and the final 45 cooling temperature are the essential process parameters. The defined cooling process step between  $Ms$  and coiling temperature is very important to realize the fine martensite microstructure and hardness of hot rolled abrasive wear resistant strips. Furthermore, to ensure microstructure and 50 mechanical properties are uniformly distributed through strip thickness and width, the water cooling on the top and bottom of strip surfaces are carefully controlled and optimised.

The final as-coiled microstructure obtained with the above 55 steel composition and process does not result in manganese banding due to the low Mn content. For the present steel composition the  $Ms$  temperature is relatively high, that is about  $400^\circ C$ , so the martensite will be auto-tempered to some extent. Therefore, the microstructure is mainly a fine martensite microstructure with small packet and block sizes transformed from the heavy deformed pancaked austenite, lower bainite and auto-tempered martensite with very fine iron carbides, and  $NbC$ ,  $Nb(C, N)$  and  $NbV(C, N)$  particles and MA islands to give the balanced properties of high 60 strength, hardness, impact toughness and bendability.

For the 450 HBW steel grade, the volume fraction of 65 martensite including auto-temperature martensite and MA

islands is at least 80% and more typically more than 90%, and the lower bainite microstructure is at most 20%, more typically at most 10% in volume fraction. For the 400 HBW steel grade, the volume fraction of martensite including auto-temperature martensite and MA islands is at least 65%, more typically more than 70% and less than 80%, and the rest of lower bainite microstructure is at most 35%, more typically at most 30% and at least 20% in volume fraction.

The key parameters of the process to produce the high strength wear resistant strip Brinell hardness above 400 HBW and low carbon equivalent values and the strip produced according to the process are the steel composition, slow cooling inside the hot box, hot rolling, fast cooling in two stages on the run-out table and low temperature coiling.

The present invention solves the problem that the carbon equivalent values (CEV, CET and Pcm) have to be increased and a different steel composition has to be applied for the higher wear resistant steel grade and thicker strips due to higher hardness requirement in higher steel grade, and the hardenability issue for the thicker hot rolled steel strips in order to maintain a similar hardness level as that of thinner hot rolled strips. Furthermore, the present invention also the problems of lower impact toughness and poorer bendability and weldability properties related to high strength high hardness wear resistant steels and high carbon equivalent values.

Some typical mechanical properties of high strength hot rolled steel strips with different thickness are shown in Table 1 below. With respect to the abrasion resistant property, the common testing standard ASTM G65—the dry sand rubber wheel abrasion test was carried out according to the procedure B—10 minutes testing time. The abrasive material is the rounded quartz grain sand, as specified as AFS 50/70 silica sand, was used for the wear testing. The wear sample weight was measured before and after wear testing with a scale to an accuracy of  $10^{-4}$  g to determine weight loss. In Table 1, the relative wear life to reference steel S355 was calculated by weight loss of S355/wear loss of different gauge of hot rolled strips.

TABLE 1

| Gauge<br>(mm) | Steel<br>Grade | Brinell<br>Hard-<br>ness |                                 | YS<br>(MPa) | UTS<br>(MPa) | Elonga-<br>tion<br>A50% | CVN<br>(-40°<br>C.) | R/t  | Rela-<br>tive<br>wear<br>life to<br>S355 |
|---------------|----------------|--------------------------|---------------------------------|-------------|--------------|-------------------------|---------------------|------|------------------------------------------|
|               |                | HBW                      | Brinell<br>Hard-<br>ness<br>HBW |             |              |                         |                     |      |                                          |
| 4             | 450<br>HBW     | 458                      | 1208                            | 1462        | 10           | N/A                     | 3                   | 2.46 |                                          |

TABLE 1-continued

| 5  | Gauge<br>(mm) | Steel<br>Grade | Brinell |                      |             |              | CVN<br>(-40°<br>C.) | R/t | Rela-<br>tive<br>wear<br>life to<br>S355 |
|----|---------------|----------------|---------|----------------------|-------------|--------------|---------------------|-----|------------------------------------------|
|    |               |                | HBW     | Hard-<br>ness<br>HBW | YS<br>(MPa) | UTS<br>(MPa) |                     |     |                                          |
| 10 | 4.8           | 450<br>HBW     | 456     | 1293                 | 1528        | 10           | N/A                 | N/A | N/A                                      |
| 10 | 5             | 450<br>HBW     | 454     | 1242                 | 1505        | 10           | N/A                 | 3   | 2.45                                     |
| 15 | 6             | 450<br>HBW     | 452     | 1258                 | 1500        | 11           | 89 J                | N/A | N/A                                      |
| 15 | 7             | 450<br>HBW     | 451     | 1245                 | 1502        | 11           | 84 J                | N/A | N/A                                      |
| 20 | 8             | 450<br>HBW     | 450     | 1219                 | 1459        | 12           | 80 J                | 2.5 | 2.37                                     |
| 20 | 8             | 400<br>HBW     | 416     | 1180                 | 1385        | 11           | 110 J               | 2   | 2.05                                     |
| 20 | 10            | 450<br>HBW     | 446     | 1221                 | 1434        | 14           | 73 J                | N/A | N/A                                      |
| 25 | 10            | 400<br>HBW     | 412     | 1162                 | 1316        | 12           | 95 J                | N/A | N/A                                      |
| 25 | 11            | 450<br>HBW     | 445     | 1183                 | 1432        | 16           | 53 J                | N/A | N/A                                      |
| 25 | 12            | 400<br>HBW     | 400     | 1121                 | 1345        | 15           | 61 J                | 2   | 1.93                                     |
| 30 | 16            | 400<br>HBW     | 400     | 1127                 | 1342        | 15           | 37 J                | 2   | 1.71                                     |

It is clearly shown in Table 1 that the abrasive wear resistant strip product has high strength ( $\geq 1500$  MPa up to a thickness of 4.2 mm), high elongation ( $\geq 10\%$ ), high toughness (e.g. for 8 mm 400 HBW grade strip, the Charpy toughness is 110 J at the  $-40^\circ$  C.). More importantly, with the present invention two different high strength wear resistant steel grades (400 HBW and 450 HBW) in a wide range of strip thickness can be produced. At the same time the wear resistant hot rolled strips have very low carbon equivalent (CEV, CET and Pcm) values, which means good weldability. The abrasive wear resistant strip also has excellent bendability and abrasive wear resistant properties.

Examples of the steel composition (Code A-M) are given in the Table 2, together with three carbon equivalent values (CEV, CET and Pcm). Please note that the boron content in these examples is about 0.0025 wt % and N content is about 0.005 wt %. The different steels of all examples are calcium treated.

TABLE 2

| Code | C    | Si   | Mn   | Cr   | Mo   | Ni   | Al   | Ti    | Cu   | Nb    | V    | Nb + V | CEV  | CET  | Pcm  |
|------|------|------|------|------|------|------|------|-------|------|-------|------|--------|------|------|------|
| A    | 0.13 | 0.03 | 1.15 | 0.35 | 0.13 | 0.07 | 0.05 | 0.020 | 0.10 | 0.030 | 0.10 | 0.13   | 0.45 | 0.28 | 0.25 |
| B    | 0.14 | 0.01 | 1.08 | 0.40 | 0.12 | 0.05 | 0.07 | 0.002 | 0.05 | 0.015 | 0.09 | 0.11   | 0.45 | 0.28 | 0.25 |
| C    | 0.15 | 0.03 | 0.88 | 0.21 | 0.20 | 0.05 | 0.06 | 0.010 | 0.06 | 0.024 | 0.12 | 0.14   | 0.41 | 0.27 | 0.25 |
| D    | 0.16 | 0.04 | 1.17 | 0.25 | 0.15 | 0.02 | 0.03 | 0.018 | 0.08 | 0.027 | 0.04 | 0.07   | 0.45 | 0.31 | 0.27 |
| E    | 0.17 | 0.04 | 1.15 | 0.05 | 0.16 | 0.05 | 0.03 | 0.016 | 0.03 | 0.015 | 0.10 | 0.12   | 0.43 | 0.31 | 0.27 |
| F    | 0.19 | 0.03 | 0.52 | 0.40 | 0.20 | 0.08 | 0.06 | 0.020 | 0.07 | 0.026 | 0.10 | 0.13   | 0.43 | 0.29 | 0.28 |
| G    | 0.19 | 0.04 | 1.00 | 0.05 | 0.15 | 0.10 | 0.04 | 0.020 | 0.09 | 0.015 | 0.05 | 0.07   | 0.42 | 0.31 | 0.28 |
| H    | 0.20 | 0.03 | 0.70 | 0.30 | 0.16 | 0.02 | 0.06 | 0.010 | 0.05 | 0.020 | 0.05 | 0.07   | 0.42 | 0.30 | 0.29 |
| I    | 0.21 | 0.04 | 0.70 | 0.20 | 0.20 | 0.02 | 0.07 | 0.002 | 0.02 | 0.025 | 0.07 | 0.10   | 0.42 | 0.31 | 0.30 |
| J    | 0.21 | 0.03 | 0.70 | 0.30 | 0.12 | 0.05 | 0.06 | 0.015 | 0.04 | 0.029 | 0.08 | 0.11   | 0.43 | 0.31 | 0.30 |
| K    | 0.22 | 0.05 | 0.75 | 0.15 | 0.11 | 0.08 | 0.07 | 0.015 | 0.05 | 0.023 | 0.06 | 0.08   | 0.42 | 0.32 | 0.30 |
| L    | 0.23 | 0.04 | 0.70 | 0.10 | 0.10 | 0.05 | 0.07 | 0.020 | 0.02 | 0.025 | 0.05 | 0.08   | 0.40 | 0.32 | 0.30 |
| M    | 0.23 | 0.04 | 0.55 | 0.20 | 0.10 | 0.07 | 0.05 | 0.020 | 0.09 | 0.020 | 0.08 | 0.10   | 0.41 | 0.31 | 0.31 |

FIG. 1 shows a SEM image (10816 $\times$  magnification) of 450 HBW grade from a 4.2 mm high strength wear resistant hot rolled steel strip. The volume fractions of the martensite content including auto-tempered martensite and MA islands, and lower bainite are depending on the target steel grades and strip thickness. In the example of FIG. 1 the volume fraction of martensite including auto-temperature martensite and MA islands is 85 $\pm$ 3%, and the rest of microstructure is lower bainite that is 15 $\pm$ 3% in volume fraction.

The invention claimed is:

1. A high strength, hot rolled abrasive wear resistant steel strip, wherein the strip has a thickness in the range of 3-20 mm and has a microstructure comprising martensite, auto-tempered martensite with iron carbides and NbC, Nb(C, N) and NbV(C, N) particles and trace amounts of retained austenite in martensite-austenite islands, with low carbon equivalent values CEV, CET and PCM and wherein the steel contains in weight percentages:

C: 0.15-0.29  
 Si: 0.01-0.05  
 Mn: 0.6-0.9  
 Cr: 0.05-0.8  
 Mo: 0.05-0.4  
 Ni: at most 0.1  
 Cu: at most 0.1  
 Al: 0.01-0.08  
 Ti: at most 0.02  
 B: at most 0.004  
 Nb: 0.005-0.035  
 V: 0.06-0.15  
 P: at most 0.020  
 S: at most 0.010  
 N: at most 0.006  
 H: at most 0.0004

Ca additions for sulphide shape control: 0.0005-0.005  
 wherein the total content of Nb+V is in a range of 0.065-0.16

other elements in amounts of impurity level, balance iron, and wherein CEV is at most 0.46, CET at most 0.34 and PCM at most 0.32, wherein the strip has a Brinell hardness of at least 400 HBW and a tensile strength of at least 1316 MPa, and wherein CEV, CET and PCM are defined as follows:

$$CEV=C+Mn/6+Cr/5+Mo/5+V/5+Cu/15+Ni/15;$$

$$CET=C+Mn/10+Mo/10+Cr/20+Cu/20+Ni/40;$$

$$PCM=C+Si/30+Mn/20+Cu/20+Cr/20+Mo/15+V/10+Ni/60+5B.$$

2. The strip according to claim 1, wherein the strip up to a thickness of 4.2 mm has a Brinell hardness of at least 458 HBW and a tensile strength of at least 1460 MPa.

3. The strip according to claim 1, wherein the strip at a thickness in the range of 3-16 mm has a Brinell hardness of at least 400 HBW and a tensile strength of at least 1316 MPa.

4. The strip according to claim 1, wherein C is in the range of 0.15-0.23 wt %.

5. The strip according to claim 1, wherein Mo is in a range of 0.05-0.25 wt %.

6. The strip according to claim 1, wherein V is in the range of 0.07-0.15 wt %.

7. The strip according to claim 1, wherein V is in a range of 0.08-0.15 wt %.

8. The strip according to claim 1, wherein V is in the range of 0.09-0.15 wt %.

9. The strip according to claim 1, wherein CEV is at most 0.43, CET is at most 0.31 and PCM is at most 0.29.

5 10. A process for producing a high strength, hot rolled abrasive wear resistant steel strip, wherein the strip has a thickness in the range of 3-20 mm and has a microstructure comprising martensite, auto-tempered martensite with iron carbides and NbC, Nb(C, N) and NbV(C, N) particles and 10 trace amounts of retained austenite in martensite-austenite islands, with low carbon equivalent values CEV, CET and PCM, comprising the steps of:

casting a slab with a composition in wt %

C: 0.15-0.29  
 Si: 0.01-0.05  
 Mn: 0.6-0.9  
 Cr: 0.05-0.8  
 Mo: 0.05-0.4  
 Ni: at most 0.1  
 Cu: at most 0.1  
 Al: 0.01-0.08  
 Ti: at most 0.02  
 B: at most 0.004  
 Nb: 0.005-0.035  
 V: 0.06-0.15  
 P: at most 0.020  
 S: at most 0.010  
 N: at most 0.006  
 H: at most 0.0004

30 Ca additions for sulphide shape control: 0.0005-0.005 and wherein the total content of Nb+V is in a range of 0.035-0.16, other elements in amounts of impurity level, balance iron, and wherein CEV, CET and PCM are defined as follows:

$$CEV=C+Mn/6+Cr/5+Mo/5+V/5+Cu/15+Ni/15;$$

$$CET=C+Mn/10+Mo/10+Cr/20+Cu/20+Ni/40;$$

$$PCM=C+Si/30+Mn/20+Cu/20+Cr/20+Mo/15+V/10+Ni/60+5B;$$

containing the slab in a hot box for a predefined time, reheating the slab to a temperature of at least 1150° C., keeping the slab for a predefined period at the temperature of at least 1150° C., and

hot rolling the slab to a hot rolled steel strip with a finish rolling temperature in the range of 800-940° C.,

water cooling the strip with a cooling rate in the range of -20-150° C./s,

coiling the strip at a temperature in the range of 100-250° C.

11. The process according to claim 10, wherein the slab is contained in the hot box for a period in the range of 2-6 days.

12. The process according to claim 10, wherein the temperature of the slab at the end of the period is in the range of 400-500° C.

13. The process according to claim 10, wherein the slab is kept at the temperature of at least 1150° C. for a period of 0.5-3 hours.

14. The process according to claim 10, wherein the slab is contained in the hot box for a period in the range of 3-5 days.